# EUROPEAN PATENT SPECIFICATION

(11) **EP 1 933 332 B1**
(45) Date of publication and mention of the grant of the patent: **15.02.2012**
(21) Application number: 07122336.6
(22) Date of filing: 05.12.2007
(51) Int. Cl.: H01B 3/18, H01B 3/44, H01B 3/02, H01F 27/32

(54) **Insulation system and method for a transformer**
Isoliersystem und Verfahren für einen Transformator
Système d'isolation et procédé pour un transformateur

(30) Priority: 15.12.2006 US 639725
(43) Date of publication of application: 18.06.2008
(73) Proprietor: GENERAL ELECTRIC COMPANY, Schenectady, NY 12345 (US)
(72) Inventor: Tan, Qi, Rexford, NY 12148 (US); Irwin, Patricia Chapman, Altamont, NY 12009 (US); Cao, Yang, Niskayuna, NY 12309 (US); Younsi, Abdelkrim, Ballston Lake, NY 12019-1022 (US)
(74) Representative: Bedford, Grant Richard

(56) References cited:
- US-A- 4 212 914
- US-A- 4 219 791

## Description

The invention relates generally to insulating systems for electrical machines and machine windings, and more specifically to an insulation system having non-linear dielectric properties.

Electrical machines and devices such as generators, motors, actuators, transformers, etc. are constantly subjected to various electrical, mechanical, thermal, and environmental stresses. Such stresses tend to degrade them, consequently reducing their lives. In an example, a static magnetic field is retained after power is disconnected in a steel core in transformers due to magnetic remanence. When power is further reapplied, residual field causes a high inrush current until effect of the magnetic remanence is reduced, usually after a few cycles of applied alternating current. Overcurrent protection devices such as fuses in transformers connected to long overhead power transmission lines are unable to protect the transformers from induced currents due to geomagnetic disturbances during solar storms that may cause saturation of the steel core, and false operation of transformer protection devices. It has been commonly observed that deterioration of insulation in the foregoing devices is a dominant factor in their failures.

Insulation systems for electrical machines such as generators, motors and transformers have been under constant development to improve performance of the machines. Materials generally used in electrical insulation include polyimide film, epoxy-glass fiber composite and mica tape. Insulating materials generally need to have the mechanical and physical properties that can withstand various electrical rigors of the electrical machines such as lightning and switching surges. In addition, some of the desirable properties of an insulation system include withstanding extreme operating temperature variations, and a long design life.

The aforementioned insulating materials have an essentially constant dielectric constant, which protects them from electrical conduction based on their respective composite breakdown strengths. However, certain factors such as operating temperatures, environment, voltage stresses, thermal cycling and voltage surges from lightning and switching deteriorate the insulating materials over a long period of time thus reducing their useful or operational life.

US 4219791 discloses an electrical inductive apparatus including an insulating dielectric surrounding a plurality of a windings. The insulating structure comprises an adhesive or binder such as organic resin filled with microspheres made of glass or silica.

US 4212914 discloses an electro-insulating material used for insulating electric windings of transformers for example. The material comprises fluorine rubber, mica-containing materials, resin, cross-linking agents and the balance being made up with a filler. Optionally, synthetic rubber is included as well.

DE 4 438 187 discloses the use of the non-linear dielectric fillers zinc oxide and silicon carbide in the insulation layers of windings for transformers.

Therefore, it would be desirable to provide an insulation system that would address the aforementioned problems and meet the current demands of industry applications.

The present invention provides a transformer according to claim 1 and a method of fcorming insulation therein according to claim 6.

Various features, aspects, and advantages of the present invention will become better understood when the following detailed description is read with reference to the accompanying drawings in which like characters represent like parts throughout the drawings, wherein:
FIG. 1 is a perspective view of a transformer including a magnetic core with windings employing a non-linear or varying dielectric material as insulation in accordance with an embodiment of the invention;
FIG. 2 is a vertical sectional view of the transformer in FIG. 1 illustrating multiple turns in the windings;
FIG. 3 is a cross-sectional view of a non-linear dielectric insulation system employed in FIG. 2 in accordance with an embodiment of the invention;
FIG. 4 is a schematic illustration of a corner of the winding of FIG. 2 experiencing electrical stress;
FIG. 5 is a graphical comparison of dielectric constant as a function of electric field intensity of polyvinylidene fluoride film without and with fillers, all of which may be used in an electrical machine and with windings in accordance with an embodiment of the invention; and
FIG. 6 is a graphical illustration of electric field strength around the corner in FIG. 4.

As discussed in detail below, various embodiments of the present invention include an insulation system using non-linear or varying dielectric property materials. As used herein, the term "non-linear" refers to a non-uniform change in dielectric constant with voltage. The insulation system disclosed herein may be employed in machines operating at high voltages such as, but not limited to, transformers. The insulation system includes an inherent adaptive property such that the dielectric constant of the non-linear dielectric may increase at locations in the machine insulation experiencing high electrical stress and provide desirable electrical protection to the machine. The electrical protection is obtained through electrical stress smoothing and reduction in the local electric field intensity.

Turning now to the drawings, FIG. 1 is a perspective view of a transformer 10 including a tank 12. The transformer 10, in the illustrated embodiment, is a three phase shell-core transformer. In another embodiment, the transformer 10 may be a single phase transformer. The transformer 10 includes a magnetic core 14 having a first core section 16 and a second core section 18 having at least one opening 20 and disposed adjacent to each other. In a particular embodiment, the first core section 16 and the second core section 18 may include three openings 20 each. The first core section 16 and the second core section 18 may also include multiple superposed laminated stacks 22. In a particular embodiment, the laminated stacks 22 may include laminated stacks made of a metal such as, but not limited to, steel. The transformer 10 may further include electrical winding phases 24, 26 and 28. Each of the electrical winding phases 24, 26 and 28 may include multiple windings 30 that are insulated by a non-linear dielectric layer (not shown) and stacked adjacent to each other. The windings 30 may surround the first core section 16 and the second core section 18 through openings 32 and the opening 20.

FIG. 2 is a vertical sectional view of the transformer 10 in FIG. 1 illustrating the windings 30. The windings 30 may include a conductive material that is wound spirally to form multiple turns 36, 38 and 40. In a particular embodiment, the conductive wire used is generally a magnet wire. Magnet wire is a copper wire with a coating of varnish or some other synthetic coating. In a non-limiting example, the number of turns may vary in the range between about a few to about thousands depending upon the power and application.

FIG. 3 is a cross-sectional view of the winding 30 in FIG. 2. Each of the turns 36, 38 and 40,as referenced in FIG. 2, include outer strands 42, 44 and 46 respectively. Similarly, the turns 36, 38 and 40 include inner strands 48, 50 and 52 respectively. The strands 42 and 48 are disposed in a row of strands in each turn 36 so that multiple turns 36, 38 and 40 may be disposed in a parallel arrangement. A non-linear dielectric insulation layer 54 may be applied around each of the outer strands 42, 44 and 46. Similarly, the non-linear dielectric insulation layer 54 may be applied around each of the inner strands 48, 50 and 52. Further, a non-linear dielectric insulation layer 56 may be applied between the turns 36, 38 and 40. In a presently contemplated embodiment, the dielectric constant of the non-linear dielectric insulation layers 54 and 56 increases with voltage or a local electric field.

In a particular embodiment, the non-linear dielectric insulation may include a mixed composite of a glass cloth, an epoxy binder, mica paper and a filler of size ranging from at least about 5 nm. Some non-limiting examples of the filler may include a micron filler and a nano filler. As noted above, such fillers may include lead zirconate, lead hafnate, lead zirconate titanate, lanthanum-doped lead zirconate stannate titanate, sodium niobate, barium titanate, strontium titanate, barium strontium titanate and lead magnesium niobate. In another example, the non-linear dielectric insulation may include polyetherimide, polyethylene, polyester, polypropylene, polytetrafluoroethylene, polyvinylidene fluoride, and polyvinylidene fluoride coploymers. Some non-limiting examples of mica may include muscovite, phlogopite, anandite, annite, biotite and bityte. The glass cloth may have varying amounts of woven density. Some non-limiting examples of the glass cloth are listed below in Table 1.

**Table 1:**

| Style | Weave | Count Warp | Yarns Fill | Weight | | Thickness | | Strength | |
|---|---|---|---|---|---|---|---|---|---|
| | | | | oz/yd^2 | g/m^2 | mils | mm | Warp Ibf/in (N/mm) | Fill Ibf/m (N/mm) |
| 1076 | Plain | 60 | 25 | 0.96 | 33 | 1.8 | 0.05 | 120 (21) | 20 (3.5) |
| 1070 | Plain | 60 | 35 | 1.05 | 36 | 2 | 0.05 | 100 (17.5) | 25 (4) |
| | | | | | | | | | |
| 6060 | Plain | 60 | 60 | 1.19 | 40 | 1.9 | 0.05 | 75 (13) | 75 (13) |
| 1080 | Plain | 60 | 47 | 1.41 | 48 | 2.2 | 0.06 | 120 (21) | 90 (16) |
| 108 | Plain | 60 | 47 | 1.43 | 48 | 2.5 | 0.06 | 80 (14) | 70 (12) |
| 1609 | Plain | 32 | 10 | 1.48 | 50 | 2.6 | 0.07 | 160 (28) | 15 (3) |
| 1280/1086 MS | Plain | 60 | 60 | 1.59 | 54 | 2.1 | 0.05 | 120 (21) | 120(21) |

Glass cloth of various woven densities, weights, thicknesses and strengths have been listed. A first example of the glass cloth is of a1076 glass type with a plain weave having a warp count of 60 and a weight of 33 g/m². Similarly, other example include 1070, 6060, 1080, 108, 1609, and 1280 glass types. Glass acts as a mechanical support for the insulation system and also adds inorganic content to the composite that improves the thermal conductivity of the final composite system. The mica acts as the primary insulation for the composite. The epoxy binder is the only organic portion of the composite insulation system and acts as the glue to hold the system together. Further, the nonlinear filler provides the nonlinear response to the insulation system as well as improving the thermal conductivity of the composite. An electrical field stress may be experienced at edges of the outer strands 42, 44 and 46 and the inner strands 48, 50 and 52. There is also a high degree of electrical field stress measured at corners of the turns 36, 38 and 40 during transformer operation. The non-linear dielectric insulation layers 54 and 56 enable a more uniform distribution of electrical field and alleviate regions experiencing high electrical stress.

There are several ways to incorporate a filler into an insulation composite. Some non-limiting examples include extrusion of the filler and polymer forming a filled polymer system, solvent dispersion of the filler and polymer with subsequent evaporation of the solvent forming a film and using screen printing or dip coating techniques for incorporating the filler into the crossover points of the warp and weft fibers of the glass cloth. Furthermore, it has been found that silane treatment such as, but not limited to, 3-Glycidoxypropyl trimethoxysilane of the filler and the glass is important to desirable adhesion of the filler to the glass cloth and final composite structure. The choice of filler incorporation method depends on the final structure of the insulation composite. In an example, filled polymer films usually use extrusion, or solvent dispersion. In another embodiment, tapes of mica, glass cloth and epoxy resin usually use screen printing or dip coating on the glass cloth technique.

FIG. 4 is an exemplary schematic illustration of electrical field stress experienced at a corner 60 of the turn 36 in the winding 30 in FIG. 2. The corner 60 may include a non-linear dielectric insulation layer 56 as referenced in FIG. 3. The corner 60 is a region on the turn 36 that may undergo maximum electrical field stress during operation. It is desirable to reduce the electrical stress. A reduction in electrical stress may increase a voltage rating of the transformer. The non-linear dielectric insulation layer 56, as referenced in FIG. 3, distributes the electrical field uniformly at the corner 60 so as to minimize stress that has occurred due to an uneven distribution of the electrical field. As the electrical field stress increases at the corner 60, the non-linear dielectric layer 56 adapts accordingly so as to provide a more uniform electrical field distribution 62 around the corner 60 than would be present if conventional uniform dielectric strength materials were used, thus protecting the turn 36 from potential electrical damage.

In another illustrated embodiment of the invention, a method 70 of forming an insulation in a transformer may be provided. An insulating layer having a dielectric constant that varies as a function of voltage or electric field may be disposed around at least a portion of a winding in step 72. In a particular embodiment, the insulating layer may be disposed around a corner of the winding. In another embodiment, the insulating layer may be disposed between multiple strands in the winding. In another embodiment, the insulating layer may be made of mica, epoxy resin, glass cloth and as ceramic filler. In yet another embodiment, the glass cloth and the ceramic filler may be coated with silane. In a presently contemplated embodiment, the ceramic filler may be attached to the glass cloth via a technique of screen printing or dip coating.

### EXAMPLES:

The examples that follow are merely illustrative and should not be construed to limit the scope of the claimed invention.

FIG. 5 is a graphical comparison 90 of dielectric constant as a function of electric field intensity for a polyvinylidene fluoride (PVDF) film without fillers and with fillers. The X-axis 92 represents electric field intensity in kV/mm. The Y-axis 94 represents dielectric constant of the PVDF film. Curve 96 represents dielectric constant of a PVDF film without a filler. As can be seen, the dielectric constant does not vary significantly as a function of the electric field intensity. Curve 98 represents dielectric constant of a PVDF film with 20% by volume of a micron lead zirconate filler. Similarly, curves 100, 102, and 104 represent dielectric constant as a function of electric field intensity for a PVDF film with 20% by volume of a nano lead zirconate filler, 40% by volume of a micron lead zirconate filler and 40% by volume of a nano lead zirconate filler respectively. As observed, the dielectric constant increases significantly from about 30 to peak at about 80 as a function of electric field intensity in the case of 40% by volume of a nano lead zirconate filler. Hence, addition of nanofillers in the PVDF film increases the variation of the dielectric constant with electrical field and enhances adaptability of an insulation system to fluctuations in electrical field stress.

FIG. 6 is a graphical illustration 110 of the electrical field profile at the corner 60 in FIG. 4 as a function of distance from a conductor such as turn 36 in FIG. 2 having a non-linear dielectric insulation layer. The X-axis 112 represents distance from the turn 36 through the non-linear dielectric insulation layer in mm. The Y-axis 114 represents electric field intensity in kilovolts/mm. As can be seen from curve 116, the electric field is stable at from 10 kV/mm with the distance from the turn 36. In electrostatics, product of the dielectric constant and electric field depends on potential difference and dielectric properties of a medium. If the dielectric constant were held constant, the local electric field on a surface adjacent to an electrically conducting element would be very high due to its relatively small area. The electric field would then decrease and reach a minimum at an outermost surface of the insulation that is at ground potential. However, if the dielectric constant were allowed to increase with the electric field, this compensating effect would force a uniformity across the entire material as shown. Thus, the non-linear dielectric insulation layer provides a generally uniform field distribution within the conductor eliminating or reducing the possibility of electrical damage to the conductor.

Beneficially, the above described insulation system and method are capable of suppressing ripple voltage and sudden current surges in transformers. Further, the suppression of transient voltages ensures a longer lifetime of operation for transformers. Usage of such insulation systems also helps in taking care of the aforementioned factors without a significant increase in size of the transformers.

While only certain features of the invention have been illustrated and described herein, many modifications and changes will occur to those skilled in the art. It is, therefore, to be understood that the appended claims are intended to cover all such modifications and changes as fall within the true spirit of the invention.

## Claims

1. A transformer (10) comprising:
a magnetic core (14) comprising a plurality of laminated stacks (22) having at least one opening; and
a plurality of windings (30) comprising a conductive material around the magnetic core (14) through the at least one opening and surrounded by an insulating layer (54) **characterised in that** the insulating layer (54) includes a filler material that provides a non-linear response to an electric field, whereby the layer has a dielectric constant that varies as a function of voltage, and the insulating layer (54) is disposed at a plurality of corners (60) of each of the plurality of windings (30).

2. The transformer (10) of claim 1, wherein the insulating layer (54) is disposed between the plurality of windings (30).

3. The transformer (10) of any preceding claim, wherein the insulating layer (54) is disposed between a plurality of strands in each of the plurality of windings (30).

4. The transformer (10) of any preceding claim, the insulating layer (54) comprising polymer composites.

5. The transformer (10) of any preceding claim, the insulating layer (54) comprising at least one nanofiller.

6. A method (70) of forming an insulation in a transformer comprising disposing an insulating layer (54) around at least a portion of a winding, **characterised in that** the insulating layer (54) includes a filler material that provides a non-linear response to an electric field, whereby the layer has a dielectric constant that varies as a function of voltage, and disposing comprises disposing the insulating layer around a corner of the winding..

7. The method (70) of claim 6, wherein disposing comprises disposing the insulating layer between a plurality of strands in the winding.

## Patentansprüche

1. Transformator (10), aufweisend:
einen magnetischen Kern (14) mit mehreren Blechpaketen (22) mit wenigstens einer Öffnung; und
mehrere Wicklungen (30), die ein leitendes Material um den Magnetkern (14) herum durch die wenigstens eine Öffnung hindurch und umgeben von einer Isolationsschicht (54) aufweisen, **dadurch gekennzeichnet, dass** die Isolationsschicht (54) ein Füllmaterial aufhält, das eine nicht-lineare Reaktion auf ein elektrisches Feld zeigt, wodurch die Schicht eine Dielektrizitätskonstante hat, die als eine Funktion der Spannung variiert, und dass die isolierende Schicht (54) an mehreren Ecken (60) von jeder der mehreren Wicklungen (30) angeordnet ist.

2. Transformator (10) nach Anspruch 1, wobei die isolierende Schicht (54) zwischen den mehreren Wicklungen (30) angeordnet ist.

3. Transformator (10) nach einem der vorstehenden Ansprüche, wobei die isolierende Schicht (54) zwischen mehreren Drähten in jeder von den mehreren Wicklungen (30) angeordnet ist.

4. Transformator (10) nach einem der vorstehenden Ansprüche, wobei die isolierende Schicht (54) Polymerverbundstoffe aufweist.

5. Transformator (10) nach einem der vorstehenden Ansprüche, wobei die isolierende Schicht (54) wenigstens ein Nanofüllmaterial aufweist.

6. Verfahren (70) zum Erzeugen einer Isolation in einem Transformator mit dem Schritt der Anordnung einer isolierenden Schicht (54), um wenigstens einen Abschnitt einer Wicklung, **dadurch gekennzeichnet, dass** die Isolationsschicht (54) ein Füllmaterial aufhält, das eine nicht-lineare Reaktion auf ein elektrisches Feld zeigt, wodurch die Schicht eine Dielektrizitätskonstante hat, die als eine Funktion von Spannung variiert, und der Schritt der Anordnung eine Anordnung der isolierenden Schicht (54) um eine Ecke der Wicklung umfasst.

7. Verfahren (70) nach Anspruch 6, wobei der Schritt der Anordnung die Anordnung der isolierenden Schicht zwischen mehreren Drähten in der Wicklung umfasst.

## Revendications

1. Transformateur (10) comportant :
un noyau magnétique (14) comprenant une pluralité d'empilements stratifiés (22) ayant au moins une ouverture ; et
une pluralité d'enroulements (30) comprenant un matériau conducteur entourant le noyau magnétique (14) à travers la/les ouvertures et entouré par une couche isolante (54), **caractérisé en ce que** la couche isolante (54) contient un matériau d'apport qui assure une réponse non linéaire à un champ électrique, grâce à quoi la couche a une constante diélectrique qui varie en fonction de la tension, et la couche isolante (54) est disposée dans une pluralité d'angles (60) de chacun des différents enroulements (30).

2. Transformateur (10) selon la revendication 1, dans lequel la couche isolante (54) est disposée entre les différents enroulements (30).

3. Transformateur (10) selon l'une quelconque des revendications précédentes, dans lequel la couche isolante (54) est disposée entre une pluralité de brins de chacun des différents enroulements (30).

4. Transformateur (10) selon l'une quelconque des revendications précédentes, la couche isolante (54) contenant des composites de polymères.

5. Transformateur (10) selon l'une quelconque des revendications précédentes, la couche isolante (54) comprenant au moins un nanofiltre.

6. Procédé (70) de formation d'une isolation dans un transformateur, comportant la disposition d'une couche isolante (54) autour d'au moins une partie d'un enroulement, **caractérisé en ce que** la couche isolante (54) contient un matériau d'apport qui assure une réponse non linéaire à un champ électrique, grâce à quoi la couche a une constante diélectrique qui varie en fonction de la tension, et la disposition consiste à disposer la couche isolante autour d'un angle de l'enroulement.

7. Procédé (70) selon la revendication 6, dans lequel la disposition consiste à disposer la couche isolante entre une pluralité de brins dans l'enroulement.
